

Patented June 1, 1926.

## UNITED STATES PATENT OFFICE.

RONALD WILD, OF HOLMESFIELD, ENGLAND, ASSIGNOR, BY MESNE ASSIGNMENTS, TO  
RUSTLESS IRON CORPORATION OF AMERICA, A CORPORATION OF MARYLAND.

## MANUFACTURE OF FERRO-ALLOYS, PARTICULARLY FERROCHROMIUM ALLOYS.

No Drawing. Application filed February 5, 1923, Serial No. 617,172, and in Great Britain March 1, 1922.

The present invention is for improvements in and relating to the manufacture of ferro-alloys, and has particular reference to the manufacture of alloys of chromium and iron, such, for example, as ferro-chrome and metal of the type commonly known as stainless or unstainable iron and steel.

For convenience the invention will be described exclusively in reference to the production of alloys of iron and chromium.

In the manufacture of metal of the class known commercially as unstainable or stainless iron and steel the alloy ferro-chrome is employed. For the production of unstainable steels this alloy may contain a substantial proportion of carbon, say 2 per cent or more, but for making unstainable chrome-iron it is the practice to use the grade of ferro-chrome known as carbon-free, i. e. ferro-chrome of a carbon content not exceeding 0.10 per cent. As the carbon-free alloy as ordinarily obtainable is comparatively costly the manufacture therefrom of stainless iron is correspondingly expensive, and the use of the latter is therefore practically restricted to articles of high or relatively high price.

Ferro-chrome is usually prepared by reduction of chromite. By effecting this reduction with an appropriate silicon-reducer it is possible to obtain directly a low carbon or carbon-free alloy, and silicon and silicides such as calcium silicide have been proposed for this purpose. The use of silicon-reducers, however, results in the production of a metal containing, according to circumstances, a varying, but generally substantial, proportion of silicon, and a process has been described in which advantage is taken of this fact in order to produce a special alloy-steel containing a comparatively high minimum percentage of this element. It is the purpose of the present invention to provide an improved and simple process for the manufacture of ferro-alloys as exemplified by ferro-chrome and stainless metal having a low content both in silicon and carbon.

According to the present invention, the manufacture of low-carbon or carbon-free ferro-alloys, such, for example, as ferro-chrome or stainless metal, by a process of the type wherein a reducible compound or compounds (such as the oxide or oxides) of a metal or metals of the alloy is or are reduced by exothermic reaction with silicon, is char-

acterized by effecting this reduction in presence of a substantial excess of the reducible compound or compounds over the quantity chemically equivalent to the reducing agent.

I have found that, in contradistinction to operating with substantially chemical equivalents of the reacting substances, the use in substantial excess of a reducible metallic compound or compounds has the effect of inhibiting the absorption of silicon by the reduced metal and that the quantity of this element thus absorbed may be so lowered as to give for all practical purposes an alloy of negligible silicon-content.

My experiments have shown that the advantageous result associated with this invention, namely, the production by silicon reduction of a product containing but a low proportion of absorbed silicon, is not to be obtained by the use of a slight excess of the reducible body or of an excess in the neighborhood of the quantity equivalent to the reducer. My experiments have shown that the production of a low-silicon product by silicon reduction is not attainable by the use of an excess of reducible oxide below a minimum of 10 to 25 per cent, according to whether a low-chromium metal (such as unstainable metal, which may contain from 9 to 20 per cent of chromium) or a high-chromium metal (such as ferro-chrome, which may contain over 70 per cent of chromium) is in course of preparation, and according as the temperature of the furnace is lower or higher, the production of a high-chromium metal requiring, other conditions remaining the same, a greater excess than when a low-chromium metal is in question, and likewise, other conditions remaining the same, a high temperature, with a more fluid slag, demands the use of a greater excess than when the temperature is lower and the slag less fluid. As will be understood, a rule for all cases is not to be laid down, and in a particular case the excess of reducible body employed must be determined by a preliminary run according to the operative conditions to be employed in the manufacture. By a "substantial excess" as referred to in this specification and in the claims is meant an excess beyond the limit of an equivalent quantity and not below the minimum percentage above mentioned. To ensure satisfactory and regular results, under operative conditions similar to those

indicated in the specification, it is, however, recommended to work with an excess well above the minimum stated, as I have shown in the specific examples hereinafter set forth.

The silicon-reducer may be ferro-silicon, preferably of high silicon-content, for instance 80-90 per cent.

The reduction may be carried out in presence of a reagent having a special affinity for oxidized silicon under furnace conditions, such, for example, as limestone or lime which combine with the silica and form a slag therewith.

Stainless chrome-iron or chrome-steel may be directly produced by effecting the reduction of a suitable oxidized compound of chromium, such as chromite, within a bath of molten iron or steel free from carbon, or of such content therein as shall provide for the desired proportion of carbon in the final alloy metal.

I prefer to utilize this direct process when manufacturing unstainable metal, because I have found that by effecting the reduction within a bath of steel in presence of a substantial excess of the reducible oxide, the absorption of silicon by the reduced metal appears to be still further inhibited, and it is possible directly to obtain a low-silicon product with a considerably lower percentage excess. Reduction of ore within a bath of steel has been previously proposed, but according to my invention this reduction is carried out in a particular way, namely, in presence of a substantial excess of the reducible oxide for the purpose and with the results aforesaid.

The reducing bath may consist essentially of a fused ferro-silicon of comparatively low silicon content, such a bath being conveniently provided by a molten charge of iron or of mild steel containing the desired proportion of a ferro-silicon of high-silicon content, for instance, one of 80 to 90 per cent. The carbon content of the ferro-silicon should be known so that allowance may be made therefor in preparing the bath according to the nature of the metal desired.

For the direct production in this manner of stainless metal various alternatives in procedure may be employed, for instance:

(a) A charge of chromite is first fused with the bath of iron or steel, the silicon-reducer added to the melt, and then a further charge of the chromite introduced in quantity substantially the chemical equivalent to the reducing agent. This second addition of chromite may be made in a single charge or in successive charges as may be desired.

Proceeding in this way, namely, by first fusing with a part of the reducible charge, the bath is brought into condition for effective subsequent reduction, and it has been found that by operating thus a product of

low content in silicon may be obtained with the subsequent employment of a quantity of the reducible compound not materially different from that equivalent to the reducing agent, with, of course, due regard to process losses.

(b) The chromite and reducing agent are heated together to a temperature approaching that of reaction, and the requisite quantity of molten iron or steel is then added to the preheated mixture, heat being subsequently applied as required to ensure completion of the reaction or the production of a homogeneous melt.

(c) A ferro-chrome is first prepared by reduction of chromite with a silicon-reducer, the addition then made to the fused alloy of molten iron or steel, preferably containing dissolved oxygen or oxides (for example, recently blown Bessemer metal), in requisite quantity to produce an alloy of the metallic composition of stainless metal and of low average content in both silicon and carbon through dilution, or dilution and oxidation, of the silicon present in the initial ferro-chrome.

The excess of the chromite or the like employed for the reduction necessarily depends upon circumstances, such as the nature of the reducible compound or the particular composition of the bath, but a simple preliminary experiment suffices to determine the most advantageous proportions of the reacting substances in a given case. Examples of an appropriate excess both in the production of ferro-chrome, and in the direct preparation of stainless chrome-iron, are given hereafter, but those acquainted with the art will readily appreciate that the excess specified in these examples can be only illustrative for the reason that with a chromite of a different composition, or with a differently constituted bath, the excess might be either greater or less than the figures given for obtaining a like result.

It will be appreciated that the content of the reducing agent in the bath determines the percentage in the final alloy of the chromium although the total charge added to the bath is not brought to the metallic state. According to circumstances, such as the furnace conditions, the yield of reduced metal varies, and as a rule will be found to be considerably less than the quantity of the metallic element theoretically obtainable from the reducible compound thereof, i. e. a process loss occurs for which allowance must be made, as will be understood by those skilled in the art. The operative details in any given case may, however, be readily determined by a simple preliminary trial.

Prior to the addition of the ferro-silicon or the like, an assay may be made of the carbon-content of the bath so that, by making allowance for the addition of the reduc-

ing agent, the carbon content may be known not to be in excess of the quantity of this element desired in the finished metal.

It is also advantageous, more particularly when manufacturing stainless iron, to fuse in the bath, prior to addition of the silicon reducer, a small proportion of a de-oxidizing reagent, such as ferro-manganese, silico-manganese, or a little ferro-silicon itself.

The process of this invention is primarily a smelting operation and may be carried out in any available furnace provided that the latter is capable of maintaining complete fusion of the materials throughout the operation of the process and of permitting the finished product to be poured or tapped into the moulds. External heating may be applied throughout or at any stage of the operations in order to maintain the requisite high temperature throughout the reduction. An electric furnace, for instance, of the Heroult or Snyder type, may conveniently be employed.

At any convenient stage of the process, the material may be submitted to an oxidizing blow, and in such case it is preferred to effect this operation according to our concurrent specification, Serial No. 617,171, that is to say, in presence of an element, (for example, manganese) more readily oxidizable than chromium at the temperature of the blowing operation. Said element may be introduced during the process of reduction as is described in concurrent specification.

The following examples will serve to indicate how the invention may be carried into effect, it being understood that these examples are given for illustrative purposes and not by way of limitation.

#### Example I.

A 5 cwt. bath of a ferro-silicon alloy was prepared by the addition to a bath of molten low-carbon steel of a high-silicon ferro-silicon (83 per cent silicon) of low carbon-content in such quantity as to give a melt containing approximately 9 per cent of silicon. A portion of the charge of the slag-forming reagent, namely, a mixture of lime and fluorspar, was added to the bath, and there were then introduced, in successive charges, 440 lbs. of chrome-iron ore, assaying 52.8 per cent of chromium sesquioxide,  $\text{Cr}_2\text{O}_3$ , and the remainder of the charge of slag-forming reagent as required to take up the oxidized silicon, to increase the fluidity of the slag and to assist in obtaining a good yield of reduced metal. The total charge of the slag-forming mixture amounted to 40 lbs. of lime and 24 lbs. of fluorspar. On completion of the reduction, a small proportion of a de-oxidizer such as manganese, ferro-manganese, or aluminium, was added according to known practice in order to ensure a sound

metal capable of casting into moulds of any desired shape. There was obtained a stainless alloy iron assaying as follows:

|            | Per cent. |    |
|------------|-----------|----|
| Chromium   | 12.95     | 70 |
| Carbon     | 0.09      |    |
| Silicon    | 0.36      |    |
| Manganese  | 0.20      |    |
| Sulphur    | 0.032     |    |
| Phosphorus | 0.046     | 75 |

The yield of stainless-iron so produced was 4 cwt. 3 qrs. 9 lbs.

It will be observed that the content of the ore in chromium sesquioxide, namely 232 lbs., was in excess of that reducible by the quantity of ferro-silicon employed, which was theoretically equivalent to about 180 lbs. of the oxide.

In like manner, ferro-alloys, such as those commonly known as stainless steel, may be prepared, the necessary higher proportion of carbon being supplied at any convenient stage of the process by the addition of suitable carbon-containing materials as are known in the art, for example, either by way of the metals employed for the initial bath or subsequently, say by the addition of the requisite quantity of pig-iron for the furnace charge, or by coal or charcoal added to the metal in the ladle.

#### Example II.

A charge of 500 lbs. of chrome-iron ore, assaying 52.8 per cent of chromium sesquioxide,  $\text{Cr}_2\text{O}_3$ , 56 lbs. of ferro-silicon (83 per cent silicon), 40 lbs. of limestone and 24 lbs. of fluorspar, was preheated to a temperature just short of that of reaction in a stock oil-fired converter wherein there were then introduced 580 lbs. of molten recently blown Bessemer metal. The reaction was completed by application of external heat, a small proportion of metallic aluminium was added, and the molten mass was run out into the moulds. There were obtained 6 1/4 cwt. of stainless-iron having the composition:

|                        | Per cent. |     |
|------------------------|-----------|-----|
| Chromium               | 12.20     |     |
| Carbon                 | 0.03      | 115 |
| Silicon                | 0.33      |     |
| Manganese              | 0.30      |     |
| Sulphur and phosphorus | 0.04      |     |

#### Example III.

A bath was made up of the following composition:—mild steel turnings 3 cwt., scrap iron 1 cwt., chrome iron ore 100 lbs., lime 40 lbs.

The mixture was brought to complete fusion, and on analysis was found to contain 0.06 per cent carbon and 0.17 per cent of chromium. There were then added 1 qr. 26 1/2 lbs. of a ferro-silicon, assaying 83.3 per cent of silicon and 0.28 per cent of carbon.

To the ferro-silicon bath so prepared were added in successive charges 300 lbs. of chrome-iron ore assaying 52.8 per cent chromium sesquioxide, the slag being tapped off from time to time. When the reaction was finished there were added 3 lbs. of ferro-manganese to bring the metal to the usual specification, and during tapping the addition was made of 2 ozs. of aluminium in accordance with the known practice for producing sound ingots.

The tapped product weighed 4 cwt. 2 qrs. 20 lbs. and assayed as follows:

|               | Per cent. |
|---------------|-----------|
| 15 Chromium   | 12.54     |
| Manganese     | 0.44      |
| Silicon       | 0.44      |
| Carbon        | 0.09      |
| Sulphur       | 0.039     |
| 20 Phosphorus | 0.011     |

Theoretically, for the quantity of ferro-silicon added and to give a silicon-remainder in accordance with the percentage composition indicated, about 155½ lbs. of chromium oxide were necessary, whereas the total charge of chrome-iron ore corresponded to 211 lbs. of this oxide. It will be seen, however, that the quantity of ore added subsequently to the addition of the ferro-silicon corresponding to 158½ lbs. of chromium oxide, that is to say, the extra quantity was approximately that chemically equivalent to the reducing agent.

35 Of the total 400 lbs. of chrome-iron ore, equivalent to 144½ lbs. of metallic chromium 65.7 lbs. of metallic chromium were produced and absorbed by the bath, the yield of metal in this instance being approximately 40 45.4 per cent of that contained in the whole of the chrome-iron ore used in the charge, and approximately 60 per cent of that contained in the ore added subsequently to the reducing agent.

#### 45 Example IV.

A bath was made up of the following composition:

|                        | Cwt. | Qrs. | Lbs. |
|------------------------|------|------|------|
| 50 Mild steel turnings | 3    | 1    | 0    |
| File steel scrap       | 1    | 1    | 0    |
| Lime                   | 0    | 2    | 0    |

This mixture was brought to complete fusion and, on assay, was found to contain 0.07 per cent of carbon. There were added 1 qr. 24 lbs. of the same ferro-silicon as before, and then, in successive charges, 3 cwt. 2 qrs. 8 lbs. of chrome-iron ore, assaying 52.8 per cent chromium sesquioxide, the slag being tapped off from time to time as required.

The addition was then made of 1 qr. 8 lbs. of Swedish white iron and 4 lbs. of ferro-manganese in order to bring the metal to the required specification, and, during tapping,

2 ozs. of metallic aluminium were added in accordance with known practice.

The tapped product weighed 4 cwt. 3 qrs. 9 lbs. and assayed as follows:

|            | Per cent. | 70 |
|------------|-----------|----|
| Chromium   | 9.86      |    |
| Manganese  | 0.18      |    |
| Silicon    | 0.14      |    |
| Carbon     | 0.16      |    |
| Sulphur    | 0.010     | 75 |
| Phosphorus | 0.009     |    |

It will be observed that the chrome-iron ore added to the reducing bath was in considerable excess over the equivalent of the ferro-silicon. Theoretically, for the quantity of ferro-silicon added and to give a silicon-remainder in accordance with the percentage composition indicated, about 153 lbs. of chromium oxide were necessary, whereas the total charge of the chrome-iron ore corresponded to 211 lbs. of this oxide, 53½ lbs. of metallic chromium were produced and absorbed by the bath, a figure corresponding to a yield of approximately 37 per cent.

The stainless metal so produced possessed in a high degree the physical attributes necessary to enable it to be deformed or shaped by forging, rolling, drop-stamping, cold drawing or pressing, and like processes commonly employed in the manufacture of objects for which metal of this type is suitable.

#### Example V.

An initial ferro-chrome was prepared by reducing a crushed and washed chromite with the calculated quantity of ferro-silicon whereby there was obtained an alloy containing 0.20 per cent of carbon and 12 per cent of silicon. To this alloy was added ferro-manganese, containing 80 per cent of manganese and 7 per cent of carbon, in such proportion as to give a metal assaying approximately:

|           | Per cent. |
|-----------|-----------|
| Chromium  | 58.50     |
| Manganese | 8.00      |
| Silicon   | 10.90     |
| Carbon    | 0.86      |
|           | 115       |

The molten mass was run into a hot converter, lined with chromite, and about four times the weight of molten recently blown Bessemer metal, free from slag, and containing approximately 0.12 per cent of oxygen was run in whereby an alloy was produced having the composition:

|           | Per cent. | 125 |
|-----------|-----------|-----|
| Chromium  | 11.70     |     |
| Manganese | 1.60      |     |
| Silicon   | 2.18      |     |
| Carbon    | 0.18      |     |

The contents of the converter were then 130

submitted to an oxidizing blow, the purified metal assaying as follows:—

|           | Per cent. |
|-----------|-----------|
| Chromium  | 12.00     |
| Manganese | 0.60      |
| Silicon   | 0.18      |
| Carbon    | 0.08      |

*Example VI.*

10 A charge of 56 lbs. of ferro-silicon, containing 83 per cent of silicon, was fused in an electric furnace of the Snyder type and there were added to the fused mass 500 lbs. of chrome-iron ore, assaying 52.8 per cent 15 of chromium sesquioxide,  $\text{Cr}_2\text{O}_3$ , together with 40 lbs. of limestone and 24 lbs. of fluor-spar, and the whole contents of the furnace were brought to complete fusion. On tapping, 145 lbs. of ferro-chrome were obtained 20 assaying:—

|          | Per cent. |
|----------|-----------|
| Chromium | 60.70     |
| Carbon   | 0.12      |
| Silicon  | 1.90      |

25 The content in chromium sesquioxide of the chrome-iron ore, namely 264 lbs. of the oxide, was in considerable excess of that reducible by the ferro-silicon which was theoretically equivalent to about 167 lbs. of the chromium oxide.

While the invention has been described with special reference to the manufacture of iron-chromium alloys of the type of ferro-chrome and stainless iron and steel, it is to be understood that I do not limit myself to this particular application and that the invention may be utilized for the production of other alloys in the manufacture of which difficulties of like nature to those presented by ferro-chrome and stainless metal are encountered. Other special metals may be present in the alloy in addition to the main special metallic component. For example, the stainless chrome metal may contain a proportion of other special metals such as nickel, tungsten, or the like, for instance, up to 2 to 3 per cent, without detriment to the stainless properties.

50 The excess of the reducible charge required for lowering the degree of silicon absorption may be furnished by a single metallic compound or by different metallic compounds, and such excess may be introduced at any convenient stage of the reduction process. For example, the process may be commenced by heating together chromite and a silicon reducer in chemically equivalent quantities and the required excess referred to provided by addition to the reaction mixture of a reducible compound of another metal (for instance, ferrous or ferric oxide) whose presence in the final alloy will either be undetimental, or is desired to pro-

vide a special metallic component. Or the 65 chromite, or other reducible compound of a special metal, may be used in part excess and the necessary balance for the total excess supplied by another appropriate reducible metallic compound.

70 Operating according to this invention it is possible readily to obtain stainless irons and steels of an average silicon content of the order of 0.14 per cent to 0.40 per cent while working under the least advantageous 75 conditions metals of this type have been obtained containing about 1.0 per cent of silicon as the maximum content in this element. I have found the unstainable metal prepared by the process of this invention to 80 be particularly free from the fault of segregation, this property manifesting itself in the divers finishing operations applied in the manufacture of articles such as knives, 85 spoons and the like, and my metal has shown itself of improved quality over like metal as usually produced by a purely melting operation. For cutlery and like uses, the steel made according to the present 90 invention may be hardened, tempered and polished in any desired manner as will be understood by those versed in the art.

95 As iron and steel of low and known carbon content are readily and cheaply obtainable, it will be seen that the invention provides a simple process for the direct production of special alloy steels and irons, as well as for the manufacture of ferro-chrome, in an expeditious and economical 100 manner.

I claim:

1. The process for the manufacture of ferro-chromium alloys which comprises bringing about an exothermic reaction between a silicon-reducer and a reducible metallic charge containing chromium, the amount of the total of said reducible metallic charge being in a substantial excess of the quantity chemically equivalent to the reducing agent.

105 2. The process for the manufacture of ferro-chromium alloys which comprises bringing about an exothermic reaction between a silicon-reducer and a reducible metallic charge containing chromium, the amount of the total of said reducible metallic charge being in a substantial excess of the quantity chemically equivalent to the reducing agent, and subjecting the molten metallic product to an oxidizing blow.

110 3. The process for the manufacture of ferro-chromium alloys which comprises reducing a reducible compound of chromium by exothermic reaction with a silicon-reducer in presence of iron and of a substantial excess of said reducible chromium compound over the quantity chemically equivalent to the reducing agent.

4. The process for the manufacture of ferro-chromium alloys which comprises reducing chromite by exothermic reaction with a silicon-reducer in presence of excess of chromite over the quantity chemically equivalent to the reducing agent.
5. The process for the manufacture of ferro-chromium alloys which comprises reducing chromite by exothermic reaction with ferro-silicon in presence of a substantial excess of chromite over the quantity chemically equivalent to the ferro-silicon.
6. The process for the manufacture of unstainable metal which comprises reducing a reducible compound of chromium by exothermic reaction with a silicon-reducer within a molten ferrous bath of a content in carbon appropriate to the desired final metal and in presence of a substantial excess of said reducible chrominum compound over the quantity chemically equivalent to the reducing agent.
7. The process for the manufacture of unstainable metal which comprises reducing a reducible compound of chromium by exothermic reaction with a silicon-reducer within a batch of low carbon steel in presence of a substantial excess of said reducible chromium compound over the quantity chemically equivalent to the reducing agent.
8. The process for the manufacture of unstainable metal which comprises the addition to a molten low silicon ferro-silicon of a reducible compound of chromium in a substantial excess of the quantity chemically equivalent to the reducing agent.
9. The process for the manufacture of unstainable metal which comprises the addition to a molten low silicon ferro-silicon of chro-
- mite in a substantial excess of the quantity chemically equivalent to the reducing agent.
10. The process for the manufacture of unstainable metal which comprises fusing ferro-silicon with low carbon steel, and then making the addition to the resulting molten low silicon ferro-silicon of chromite in a substantial excess of the quantity chemically equivalent to the ferro-silicon.
11. The process for the manufacture of unstainable metal which comprises heating ferro-silicon with chromite in a substantial excess of the quantity chemically equivalent to the ferro-silicon to a temperature approaching that of reaction and incorporating in suitable proportion with the so heated mixture a molten ferrous bath of a carbon content appropriate to the desired final metal.
12. The process for the manufacture of unstainable metal which comprises reducing chromite by exothermic reaction with a silicon reducer within a molten ferrous bath with a content in carbon appropriate to the desired final metal and in presence of a substantial excess of chromite over the quantity chemically equivalent to the reducing agent.
13. The process for the manufacture of unstainable metal which comprises reducing chromite by exothermic reaction with a silicon reducer within a bath of low-carbon steel in presence of a substantial excess of chromite over the quantity chemically equivalent to the reducing agent.

In testimony whereof I have signed my name to this specification.

RONALD WILD.

**CERTIFICATE OF CORRECTION.**

Patent No. 1,586,591.

Granted June 1, 1926, to

RONALD WILD.

It is hereby certified that error appears in the printed specification of the above numbered patent requiring correction as follows: Page 6, line 4, claim 4, after the word "of" first occurrence insert the article and word "a substantial"; and that the said Letters Patent should be read with this correction therein that the same may conform to the record of the case in the Patent Office.

Signed and sealed this 23rd day of October, A. D. 1928.

(Seal)

M. J. Moore,  
Acting Commissioner of Patents.